

# UNITED STATES PATENT OFFICE.

GUSTAV ADOLF WALDINGER AND CARL FRIEDRICH ISERLOTH, OF ELBERFELD, GERMANY,  
ASSIGNÖRS TO FARBENFABRIKEN VORM. FRIEDR. BAYER & CO., OF ELBERFELD, GER-  
MANY, A CORPORATION OF GERMANY.

## PROCESS OF DYEING.

No. 882,543.

Specification of Letters Patent. Patented March 17, 1908.

Original application filed December 29, 1906, Serial No. 349,973. Divided and this application filed June 7, 1907.  
Serial No. 377,763.

*To all whom it may concern:*

Be it known that we, GUSTAV ADOLF WALDINGER and CARL FRIEDRICH ISERLOTH, citizens of the German Empire, residing at 5 Elberfeld, Germany, Kingdom of Prussia, have invented new and useful Improvements in Process of Dyeing, of which the following is a specification.

In French Letters Patent No. 367,921, filed July 9, 1906, a process for dyeing vegetable fibers with sulfur coloring matters is described, which process consists in dyeing with these dyestuffs, in baths prepared in the usual way with the aid of alkaline sulfur 10 fids and sulfur coloring matters, but with the addition of ammonium salts. By this process level and uniform shades are obtained which in many cases are even deeper 15 and faster to washing than those obtained 20 without the employment of ammonium salts.

The present application is a divisional application from our application, Serial No. 349,973, filed December 29, 1906, and covers specifically the process for dyeing vegetable fibers with sulfur coloring matters, under 25 the addition of acids.

We have found that this favorable action of the ammonium salts seems to be due to the fact that the ammonium salts neutralize the free alkali present in the alkaline sulfur 30 sulfid dye-bath, and that acids will produce the same result. The acids are generally added to the baths in such quantities that a distinct smell of  $H_2S$  is evolved, but care 35 must be taken that no dyestuff or leuco-compound is precipitated.

The new process is also suitable for dyeing by machinery.

In order to illustrate the new process more 40 fully, the following example is given, the

parts being by weight: A dye-bath is prepared from 2000 parts of water, 10 parts of Katigen indigo B extra, 20 parts of crystallized sodium sulfid, 20 parts of Glaubers' salt, and 5 parts of soda. To this dye-bath 45 3 parts of sulfuric acid are added, and 100 parts of cotton yarn are then dyed in this bath at 50 degrees C. for 3/4 hour. The dyed goods are squeezed out, exposed to the air and rinsed. 50

The process is the same for other dyestuffs, and other acids, capable of binding alkali, such as acetic acid, or the like, may be used. The quantities added ought to be sufficient to neutralize the free alkali, but 55 care must be taken not to add an excess, and to avoid the precipitation of the dye-stuff.

Having now described our invention and in what manner the same is to be performed, 60 what we claim, is:

1. The herein-described process for dyeing the vegetable fiber with sulfur dyestuffs, which process consists in dyeing the fiber in a sulfur dyestuff bath in the presence of an 65 acid, substantially as described.

2. The herein-described process for dyeing the vegetable fiber with sulfur dyestuffs, which process consists in dyeing the fiber in a sulfur dyestuff bath in the presence of sul- 70 furic acid, substantially as described.

In testimony whereof we have hereunto set our hands in the presence of two subscribing witnesses.

GUSTAV ADOLF WALDINGER. [L. S.]  
CARL FRIEDRICH ISERLOTH. [L. S.]

Witnesses:

OTTO KÖNIG,  
OSKAR KLUG.